

May 15, 1973

TADASHI NISHI ET AL

3,733,195

CORROSION RESISTANT STEELS HAVING IMPROVED WELDABILITY

Filed Jan. 14, 1970

2 Sheets-Sheet 1



FIG. 1



FIG. 2

INVENTORS  
TADASHI NISHI  
TUNEYASU WATANABE  
HARUO SHIMADA  
HIROKI MASUMOTO  
TAKESHI FUJIMOTO  
KAZUHIRO MIIDA  
TAKASHI OKAZAKI

BY *Wenderoth, Lind & Ponack*  
ATTORNEYS

May 15, 1973

TADASHI NISHI ET AL

3,733,195

CORROSION RESISTANT STEELS HAVING IMPROVED WELDABILITY

Filed Jan. 14, 1970

2 Sheets-Sheet 2



FIG. 3

INVENTORS  
TADASHI NISHI  
TUNEYASU WATANABE  
HARUO SHIMADA  
HIROKI MASUMOTO  
TAKESHI FUJIMOTO  
KAZUHIRO MIIDA  
TAKASHI OKAZAKI

BY *Wenderoth, Lund & Ponack*  
ATTORNEYS

## 1

3,733,195

### CORROSION RESISTANT STEELS HAVING IMPROVED WELDABILITY

Tadashi Nishi, Tuneyasu Watanabe, Haruo Shimada, Hiroki Masumoto, Takeshi Fujimoto, Kazuhiro Miida, and Takashi Okazaki, Kitakyushu, Japan, assignors to Nippon Steel Corporation, Tokyo, Japan

Filed Jan. 14, 1970, Ser. No. 2,695

Claims priority, application Japan, Jan. 16, 1969, 44/3,003; Feb. 28, 1969, 44/15,630

Int. Cl. C22c 39/54

U.S. Cl. 75—125

2 Claims

### ABSTRACT OF THE DISCLOSURE

A corrosion resistant steel having improved weldability consists of 0.001–0.30 percent carbon, 0.1–2.0 percent silicon, 0.3–2.0 percent manganese, 0.01–0.50 percent chromium, 0.1–0.29 percent copper, 0.0001–0.040 percent phosphorus, two or more elements selected from the group consisting of arsenic, beryllium, bismuth, lead, germanium, antimony, selenium and tellurium in an amount of 0.02–0.20 percent each, balance being iron and unavoidable impurities. The steel may also include one or more elements selected from the group consisting of titanium, zirconium, niobium, vanadium, molybdenum, tungsten and nickel in an amount of 0.01–0.50 percent in respect to titanium, zirconium, niobium

celeration of corrosion, electrolytic aqueous solution, such as sea-water and plain water contained in the crude oil plays an important role. Further acceleration of corrosion is effected by presence of sludge and bacteria in the crude oil.

In such marine applications as above, the corrosion of steel materials is due to the physiological action of sulphate-reducing bacteria during the reduction of sulphate ions contained in the sea-water into sulphur, and thus the corrosion mechanism is quite different from those of ordinary weather-resistant steel materials (particularly corrosion by industrial atmospheres) and is characterized by severe local corrosion and pit corrosion. This is the very reason why steel materials having only weather-resistance alone cannot be used as sea-water resistant steel materials.

Presently, cathodic protection by using galvanic anode drainage using zinc, aluminium, magnesium etc. and corrosion inhibitors have been proposed for preventing such types of corrosion as above. But, all of these methods are only temporarily effective and require very large cost and labour for maintenance.

Further, steels as shown in Table 1 have been proposed for such marine applications, which are improved in sea-water resistance as well as in mechanical properties by addition of phosphorus, copper, chromium, and aluminum.

TABLE 1

| C     | Si    | Mn      | P         | S      | Cu       | Cr      | Percent of—   |           |
|-------|-------|---------|-----------|--------|----------|---------|---------------|-----------|
|       |       |         |           |        |          |         | Others        | (percent) |
| ≤0.20 | ≤0.50 | ≤0.90   | 0.07–0.15 | ≤0.04  | 0.02–0.6 | 0.2–0.8 |               |           |
| ≤0.22 | ≤0.10 | 0.6–0.9 | 0.08–0.15 | ≤0.04  | ≥0.5     | —       | Ni: 0.40–0.65 |           |
| ≥0.18 | ≥0.50 | ≤0.6    | 0.08–0.15 | ≤0.03  | 0.6–1.5  | 0.5–3.0 | Al: 0.5–1.5   |           |
| ≤0.13 | ≤0.50 | ≤0.5    | ≤0.08     | ≤0.025 | —        | 3.9–4.3 | Al: 0.7–1.1   |           |

and vanadium, 0.1–1.5 percent in respect to molybdenum and tungsten and 0.1–3.5 percent in respect to nickel, 40 balance being iron and unavoidable impurities.

### BACKGROUND OF INVENTION

Conventional sea-water resistant steels have the following corrosion problems.

(1) In case of marine structures such as base piles and buoys which are exposed and splashed with sea-water the corrosion of portions splashed with sea-water is as high as 3 to 7 times the corrosion of other portions (portions that are in the sea-water above sea), the corroded surface conditions are characterized by severe local corrosions and pin corrosions, and the corrosion products (rust) of the splashed portions have remarkable tendency of sticking as compared with the other portions.

(2) In case of applications such as marine steel piping and floats which are immersed always in the sea-water, severe corrosion takes place particularly on portions of the structure which are 1–3 m. below the sea surface. This is due to the physiological action of sulphate-reducing bacteria which reduces sulphate ions in the sea-water into sulphur and corrode the steel remarkably. This action is greater in contaminated zones and warm districts of the sea.

(3) In case of applications such as oil tankers, oil pipe lines which are exposed alternately or simultaneously with the sea-water and oils.

The corrosion is a complicated combination of whole-surface corrosions and local corrosions, the corrosion rate of the latter type being extraordinarily high. In general, corrosion in crude oil alone is very small, and for ac-

The above conventional sea-water resistant steels are improved in sea-water resistance chiefly by the addition of phosphorus and/or copper, but these additives present a critical defect that cracks at welded portions are remarkably increased in welded structures such as submarine pipe lines and buoys.

Further, many trials have been proposed for improving sea-water resistance of steels by the addition of special elements. For example, Hudson teaches in Journal of Iron and Steel Institute (JISI), 1955, July, vol. 180, pp. 271–284 that chromium, phosphorus, silicon, aluminum, molybdenum, nickel and beryllium are useful while tin, antimony, arsenic, bismuth, lead, tungsten, niobium and vanadium are not useful.

However, Hudson's findings are limited to results obtained from studies on corrosions in sea-water and in plain water, and does not teach of corrosions caused by repeated splashing of the sea-water or corrosions under a condition where both crude oil and sea-water are present. The type and mechanism of corrosion under such conditions are quite different from those in sea-water or in plain water.

### DESCRIPTION OF INVENTION

The present invention relates to corrosion resistance steels, particularly sea-water resistant steels, having improved weldability, useful for applications such as ship hulls, buoys, landing piers, base piles, dolphins (marine oil drilling platforms) which are exposed to splashing of sea-water; such as marine or submarine steel pipes and floats which are always immersed in the sea-water; and such as parts of ship hulls and oil pipe lines which are exposed alternately or simultaneously to oils, sea-water and plain water.

## 2

The basic composition of the present inventive steels comprises 0.001–0.25 percent by weight of carbon 0.1–2.0 percent by weight of silicon, 0.3–2.0 percent by weight of manganese, 0.01–3.0 percent by weight of chromium, 0.1–0.29 percent by weight of copper, less than 0.044 percent by weight of phosphorus and the balance being iron and unavoidable impurities (hereinafter "percent by weight" is abridged as "%").

The present invention will be described referring to the attached drawings in which:

FIG. 1 is a graph showing effects additions of silicon, manganese and chromium on corrosion rates in a sea-water splashing zone. FIG. 2 is a perspective view of a test piece used for the weld-crack test in Example 3, and FIG. 3 is a graph showing results of the weld-crack tests on test pieces such as shown in FIG. 2 obtained from the conventional steels and inventive steels.

One type of a preferred composition of the present inventive steels comprises: 0.001–0.25% of carbon, 0.8–1.1% of silicon, 0.3–2.0% of manganese, 0.05–3.0% of chromium, 0.1–0.29% of copper, less than 0.04% of phosphorus, the balance being iron and unavoidable impurities, in which the phosphorus and/or copper content in the conventional steels have been substituted by a combined effect of Si-Mn-Cr for eliminating welding cracks and improving sea-water resistance.

In the above preferred type of composition, reasons for limitation of each of the elements are as follows:

Silicon and manganese are well known as elements necessary for deoxidation in steel production, and chromium and copper are well known as elements necessary for improving strength and weather-resistance of steels.

However, in the present invention, when these elements are present in suitable amounts, a remarkably improved corrosion resistance which cannot be expected from the addition of one of these elements can be obtained.

For example, when both silicon and chromium are present in the steel, corrosion in a contaminated sea-water is remarkably reduced. This effect increases as the content of silicon and chromium increases, thus reducing the corrosion, including pit corrosion.

Particularly, an increased content of silicon is effective for forming a silicate film on the surface of the corrosion product (metal oxides) and is thus effective for preventing corrosion action of the sulfate-reducing bacteria in the sea-water.

However, as shown in FIG. 1, it is desirable in the sea-water splashing zone where the amount and rate of corrosion are large that the contents of both silicon and manganese are high while the content of chromium is low. The corrosion in this sea-water splashing zone is not stabilized in spite of a similar silicate film as above, but rather accelerated by a potential difference (or local electrode effects) between the base metal and the carbides of manganese and chromium formed by the corrosion. Therefore, the content of manganese is increased to reduce the corrosion or the content of chromium is lowered to prevent the carbide formation.

The present inventive steel having a composition as above shows an excellent sea-water resistance in the contaminated sea zone or in the sea-water splashing zone, and the proportion range of each element is defined as above because a steel having a composition in the above range is useful from the points of corrosion resistance, manufacturing, mechanical properties and weldability.

Namely, carbon is an element necessary for required strength of the present inventive steel. However, more than 0.25% of carbon causes embrittlement of the steel and lowers weldability and sea-water resistance, while less than 0.001% of carbon lowers steel strength and gives poor economy and productivity caused by a longer refining time. Silicon is necessary for deoxidation in the steel production, and 0.8–1.1% of silicon in combination with chromium and manganese improves sea-water

resistance. Manganese is useful as a deoxidizer and desulfurizer in steel production and is useful for improving steel strength. In the present inventive steel more than 0.3% of manganese is necessary for the required strength, but too much manganese will cause embrittlement of the steel and is thus limited to 2.0%. Copper is useful for improving sea-water resistance. This effect cannot be expected with less than 0.1% of copper, and more than 0.29% of copper will cause embrittlement and lowers weldability without any remarkable improvement in sea-water resistance. Therefore, the content of copper is limited to 0.1–0.29%. An excess amount of phosphorus embrittles the steel, and severely deteriorates joint portions of welded structures such as submarine pipe lines and buoys. Thus the upper limit of phosphorus is 0.04%. Sulphur, an unavoidable impurity, severely lowers sea-water resistance and weldability, and should be maintained as low as possible. A permissible upper limit of sulphur is 0.035%.

A second preferred composition according to the present invention comprises 0.001–0.25% of carbon, 0.1–2.0% of silicon, 0.3–2.0% of manganese, 0.01–0.5% of chromium (excluding 0.5%), 0.1–0.29% of copper, 0.001–0.040% of phosphorus, 0.02–0.20% of two or more elements selected from the group consisting of arsenic, tin, beryllium, bismuth, lead, germanium, antimony, selenium, and tellurium, and the balance being iron and unavoidable impurities.

A third preferred composition according to the present invention comprises, in addition to the second type of preferred composition, one or more elements selected from the group consisting of titanium, zirconium, niobium, vanadium, molybdenum, tungsten, and nickel and in an amount of 0.01–0.50% in respect to titanium, zirconium, niobium, and vanadium alone or in combination; 0.1–1.5% in respect to molybdenum, and tungsten in single or in combination; 0.1–3.5% in respect to nickel.

For the second and third preferred composition according to the present inventions, addition of the second group of alloying elements (titanium, zirconium, niobium, vanadium, molybdenum, nickel and tungsten) or addition of the first group of alloying elements (arsenic, antimony, tin, lead, selenium, tellurium, bismuth, beryllium and germanium) is useful to some degree for the desired corrosion resistance, but addition of these two groups of alloying elements in combination give remarkably improved and unique corrosion resistance which cannot be expected from the addition of either of the two groups alone.

The elements of the second group by themselves are effective to reduce hydrogen embrittlement, prevent intergranular corrosion and improve corrosion fatigue, but their effects are remarkably enhanced when added in combination of the elements of the first group. This is due to the fact that the elements of the first group lower the activity coefficient of nitrides or carbides of elements of the second group to convert them into a useful state and give a strong protection against severe corrosion from the co-presence of crude oil and sea-water, as well as remarkably reduce corrosion on the portions splashed with the sea-water and corrosion by bacteria in the contaminated sea zone.

The addition of the first group of elements by themselves is effective to reduce corrosion due to their toxicity to bacteria. Their effects are increased two-fold when added in combination with the second group elements, and further a remarkably improved resistance against local corrosion is given by a unique effect which reduces the ability of corrosion products to form a cathode. Particularly, chromium and silicon used with the second group elements are useful for the above combined effect. Silicon and manganese used with the second group elements have a specific ability to remarkably reduce corrosion on the portions splashed with the sea-water or corrosion under the condition where the crude oil and the sea-water are present, particularly when added in combina-

tion with copper and nickel, as in the third composition. Therefore, in view of economy, productivity, and practical utility, silicon, chromium, manganese and copper are indispensable elements in the present invention. Nickel is effective to give over-all resistance against corrosion and improve toughness at low temperatures. As for carbon and phosphorus, they are necessary for desired workability and weldability.

Thus second type of the present inventive steel has a basic composition comprising 0.001-0.25% of carbon, 0.1-2.0% of silicon, 0.3-2.0% of manganese, 0.01-0.50% of chromium, 0.1-0.29% of copper, 0.001-0.040% of phosphorus, the balance being iron, with addition of 0.02-0.20% of two or more elements selected from the first group of alloying elements to give excellent weldability. The reason for addition of two or more elements of the first group of alloys is that although the addition of arsenic alone, for example, gives good corrosion resistance, such element cannot be added in a large amount in view of weldability and mechanical properties. On the other hand, with addition of a decreased amount of arsenic together with another element of the group such as tin, improved weldability can be obtained without sacrifice of corrosion resistance. Thus, taking one consideration with another, it is advantageous to add two or more of the second group of alloying elements.

The present inventive steels having a composition as defined above may be used "as hot rolled," "as annealed" or "as tempered."

The present invention will be better understood from the following examples.

Example 1: (First type of inventive steels)

Table 2 shows results of corrosion tests under similar service conditions as met by ordinary marine constructions made on the present inventive steels and conventional steels produced in a converter, cast into ingots and hot rolled. In the table, (A) in the column of sea-water resistance shows corrosion rates after rust removal in the sea-water splashing zone determined on specimens of 50 mm. thickness x 100 mm. width x 4000 mm. length, polished on all surface with No. 160 emery, immersed 2500 mm. in the sea-water with 1500 mm. over the average water level of ebb and flow for one year, and (B) shows corrosion rates after rust removal in the contaminated sea zone, determined on specimens of 5 mm. thickness x 50 mm. width x 100 mm. length, polished on all surface with No. 600 emery, immersed 1 m. below the sea surface for one year. The corrosion rate is percent of the weight loss of the specimens to that of an ordinary carbon steel.

TABLE 2

| Number of specimens        | Chemical composition (percent) |     |      |      |      |     |       |       | Sea-water resistance rate (percent) |     |
|----------------------------|--------------------------------|-----|------|------|------|-----|-------|-------|-------------------------------------|-----|
|                            | C                              | Si  | Mn   | P    | S    | Cu  | Cr    | Ni    | A                                   | B   |
| Ordinary carbon steel..... | .18                            | .05 | .61  | .016 | .023 | .08 | ----- | ----- | 100                                 | 100 |
| Conventional steel:        |                                |     |      |      |      |     |       |       |                                     |     |
| 1.....                     | .28                            | .03 | .77  | .108 | .014 | .30 | ----- | .40   | 62                                  | 81  |
| 2.....                     | .08                            | .32 | .60  | .017 | .023 | .20 | ----- | ----- | 90                                  | 88  |
| 3.....                     | .14                            | .04 | .69  | .083 | .016 | .21 | ----- | ----- | 69                                  | 74  |
| 4.....                     | .09                            | .03 | .71  | .044 | .017 | .24 | ----- | ----- | 91                                  | 92  |
| 5.....                     | .10                            | .31 | .62  | .019 | .021 | .22 | .80   | ----- | 87                                  | 82  |
| 6.....                     | .12                            | .35 | .58  | .020 | .018 | .19 | .81   | ----- | 80                                  | 63  |
| 7.....                     | .07                            | .68 | .64  | .018 | .022 | .23 | .78   | ----- | 77                                  | 56  |
| Inventive steel:           |                                |     |      |      |      |     |       |       |                                     |     |
| 1.....                     | .12                            | .82 | .61  | .016 | .017 | .21 | .28   | ----- | 56                                  | 51  |
| 2.....                     | .13                            | .81 | .74  | .017 | .015 | .20 | .54   | ----- | 54                                  | 53  |
| 3.....                     | .10                            | .93 | .62  | .015 | .018 | .23 | .100  | ----- | 68                                  | 59  |
| 4.....                     | .10                            | .83 | .70  | .018 | .018 | .22 | .200  | ----- | 75                                  | 48  |
| 5.....                     | .10                            | .98 | 1.17 | .019 | .014 | .23 | .25   | ----- | 48                                  | 51  |

The third type of steel of the present invention further comprises, in addition to the above composition, one or more elements selected from the second group of alloying elements in amounts of 0.01-0.50% in respect to Ti, Zr, Nb, and V, 0.1-1.5% in respect to Mo and W, and 0.1-3.5% in respect to Ni to give further improved corrosion resistance and mechanical properties. The lower limits of the above additional elements are shown as limits for tangible resistance against corrosion, while the upper limits are shown as limits beyond which detrimental effects begin to appear on steel-making, or mechanical properties such as weldability and other practical properties.

For example, silicon is necessary for steel-making and in combination of chromium improves corrosion resistance. For this 0.1-2.0% of silicon is necessary. As for chromium, 0.01-0.5% is necessary for similar effects as silicon. Copper content less than 0.09% gave no tangible improvement in corrosion resistance while more than 0.2% of copper causes local corrosion and crackings and lowers weldability. Regarding the carbon content, more than 0.3% of carbon embrittles the steel and lowers weldability and corrosion resistance and further workability, while less than 0.001% of carbon lowers strength and requires a longer time of refining and deteriorates economy and productivity. As for phosphorus, more than 0.04% of phosphorus embrittles the steel and lowers weldability remarkably.

The unavoidable impurities such as sulphur have severely detrimental effects on corrosion resistance and weldability, and thus should be maintained as low as possible, and should be limited up to 0.35%.

From Table 2, it is clear that the present inventive steels show better corrosion resistance in either of the corrosive circumstances than the conventional sea-water resistant steels.

Particularly in the contaminated sea zone, the present inventive steel No. 4 which contains increased amount of Si and Cr shows excellent corrosion resistance, and in the sea-water splashing zone the present inventive steel No. 5 containing increased amount of Si and Mn with lowered chromium content show excellent corrosion resistance.

Example 2: (Second and third types of inventive steels)

Table 3 shows similarly results of corrosion tests on the present inventive steels and conventional steels produced in a converter, cast into ingots and hot rolled.

(A) In the column of sea-water resistance in Table 3 shows corrosion rates after rust removal in the sea-water splashing zone determined in the same way as (A) in Table 2, and (B) shows corrosion rates after rust removal in a sea zone near a contaminated sea zone determined in the same way as (B) in Table 2. (C) In Table 3 shows corrosion rates after rust removal determined on the specimens of 4 mm. thickness x 50 mm. width x 100 mm. length, polished on all surface with No. 320 emery and immersed horizontally for one month alternately in a tank filled with crude oil and then in a tank filled with the sea-water. As seen from the table, the present inventive steels show excellent corrosion resistance in any of the corrosion circumferences.

TABLE 3

| Number of specimens      | Chemical composition |      |      |      |      |     |     |     |     |     | Sea-water resistance corrosion rate (percent) |    |    |    |    |    |        |     |     |     |
|--------------------------|----------------------|------|------|------|------|-----|-----|-----|-----|-----|-----------------------------------------------|----|----|----|----|----|--------|-----|-----|-----|
|                          | C                    | Si   | Mn   | P    | S    | Cu  | Cr  | As  | Sn  | Sb  | Se                                            | Tu | Be | Bi | Pb | Ge | Others | A   | B   | C   |
| Ordinary carbon steel #1 | .18                  | .05  | .016 | .023 | .08  |     |     |     |     |     |                                               |    |    |    |    |    |        | 100 | 100 | 100 |
| Conventional steel #2    | .23                  | .03  | .77  | .126 | .014 | .49 |     |     |     |     |                                               |    |    |    |    |    |        | 52  | 81  | 73  |
| Conventional steel #3    |                      |      |      |      |      |     |     |     |     |     |                                               |    |    |    |    |    | Ni=.40 |     |     |     |
| Inventive steels:        |                      |      |      |      |      |     |     |     |     |     |                                               |    |    |    |    |    |        | 53  | 53  | 54  |
| 3                        | .07                  | .89  | .54  | .005 | .013 | .21 | .46 | .02 | .02 | .01 | .02                                           |    |    |    |    |    |        | 43  | 53  | 51  |
| 4                        | .16                  | .49  | 1.00 | .009 | .013 | .23 | .35 | .02 | .02 | .01 | .02                                           |    |    |    |    |    |        | 43  | 47  | 51  |
| 5                        | .07                  | .90  | 1.21 | .016 | .014 | .24 | .34 | .05 | .05 | .03 | .02                                           |    |    |    |    |    |        | 43  | 47  | 53  |
| 6                        | .65                  | .99  | 1.08 | .014 | .014 | .21 | .35 | .02 | .02 | .01 | .02                                           |    |    |    |    |    |        | 39  | 56  | 60  |
| 7                        | .20                  | .55  | .15  | .006 | .011 | .23 | .28 | .03 | .03 | .02 | .02                                           |    |    |    |    |    |        | 37  | 53  | 53  |
| 8                        | .07                  | 1.10 | 1.45 | .013 | .017 | .25 | .10 |     |     |     |                                               |    |    |    |    |    |        | 34  | 47  | 48  |
| 9                        | .11                  | .03  | .50  | .007 | .018 | .24 | .40 | .03 | .02 |     |                                               |    |    |    |    |    |        | 41  | 42  | 42  |
| 10                       | .10                  | .93  | .60  | .005 | .011 | .22 | .43 |     |     |     |                                               |    |    |    |    |    |        | 39  | 42  | 61  |
| 11                       | .13                  | .73  | .009 | .014 | .25  | .43 |     |     |     |     |                                               |    |    |    |    |    |        | 41  | 39  | 59  |
| 12                       | .09                  | 1.04 | .40  | .009 | .018 | .21 | .40 | .03 | .03 |     |                                               |    |    |    |    |    |        | 36  | 39  | 57  |
| 13                       | .12                  | .95  | .52  | .006 | .015 | .23 | .47 |     |     |     |                                               |    |    |    |    |    |        | 39  | 36  | 60  |
| 14                       | .10                  | 1.05 | .68  | .008 | .019 | .20 | .32 | .03 | .03 |     |                                               |    |    |    |    |    |        | 40  | 39  | 58  |
| 15                       | .08                  | .87  | .51  | .005 | .016 | .19 | .40 |     |     |     |                                               |    |    |    |    |    | 31     | 33  | 51  |     |
|                          |                      |      |      |      |      |     |     |     |     |     |                                               |    |    |    |    |    | Mo=.45 |     |     |     |
|                          |                      |      |      |      |      |     |     |     |     |     |                                               |    |    |    |    |    | .02    |     |     |     |

## Example 3

Specimens of 16 mm. thickness prepared from No. 2 and No. 6 steels in Table 3 were welded into the cross type fillet weld-cracking test pieces as shown in FIG. 2 with different welding current densities and speeds, and visual cracking tests were made at 10 points in the depthwise direction of the weld beads. FIG. 3 shows the results and each point in the figure shows the crack length in the bead expressed in rates to the total length of detection.

It is clear from the above test results that the present inventive steel gives stabilized weldability at high current and high speed welding conditions under which the conventional steels are encountered with crackings. What is claimed is:

1. A corrosion resistant steel having improved weldability, consisting of 0.001-0.30 percent of carbon, 0.1-

2.0 percent of silicon, 0.3-2.0 percent of manganese, 0.01-0.50 percent of chromium, 0.1-0.29 percent of copper, 0.001-0.040 percent of phosphorus, two or more elements selected from the group consisting of arsenic, beryllium, bismuth, lead, germanium, antimony, selenium and tellurium in an amount of 0.02-0.20 percent each, balance being iron and unavoidable impurities.

2. A corrosion resistant steel having improved weldability, consisting of 0.001-0.30 percent of carbon, 0.1-2.0 percent of silicon, 0.3-2.0 percent of manganese, 0.01-0.50 percent of chromium, 0.10-0.29 percent of copper, 0.001-0.040 percent of phosphorus, two or more elements selected from the group consisting of arsenic, beryllium, bismuth, lead, germanium, antimony, selenium and tellurium in an amount of 0.02-0.20 percent each, one or more elements selected from the group consisting of titanium, zirconium, niobium, vanadium, molyb-

dium, tungsten and nickel in an amount of 0.01-0.50 percent in respect to titanium, zirconium, niobium and vanadium, 0.1-1.5 percent in respect to molybdenum and tungsten and 0.1-3.5 percent in respect to nickel, balance being iron and unavoidable impurities.

## References Cited

| UNITED STATES PATENTS                        |
|----------------------------------------------|
| 3,290,183 12/1966 Ohtake - 75-126 R          |
| 2,495,854 1/1950 Marburg - 75-125            |
| 3,459,538 8/1969 Teramae - 75-126 N <b>8</b> |
| 3,278,346 10/1969 Goss - 75-125              |
| 3,328,211 6/1967 Nakamura - 75-126 F         |
| HYLAND BIZOT, Primary Examiner               |
| U.S. Cl. X.R.                                |
| 75-126 M, 126 N, 126 R                       |